

May 27, 1930.

G. W. PARKER

1,760,861

METHOD OF MAKING REFRACTORY BLOCKS

Filed May 7, 1928



FIG. 13



FIG. 10



INVENTOR  
GEORGE W. PARKER  
By Edward E. Longene  
ATTY.

## UNITED STATES PATENT OFFICE

GEORGE W. PARKER, OF ST. LOUIS, MISSOURI

## METHOD OF MAKING REFRACTORY BLOCKS

Application filed May 7, 1928. Serial No. 275,599.

My invention relates to improvements in the method of making refractory blocks, and has for its primary object to produce a refractory block for use in rotary kilns of all kinds and also in water gas generators, producer gas generators, boiler furnace walls, industrial furnace walls, and the like.

A further object is to construct a refractory block in such a manner that the exposed 10 or wearing surface is toughened.

A still further object is the method of making refractory blocks in such a manner that the grain formed during the kneading of the clay will run at right angles to the wearing 15 face of the block thereby rendering the block tougher and less liable to chip or tear out when clinkers are removed. I have discovered by hand kneading the clay prior to molding that, during the formation and kneading 20 of the wauk, a grain is formed similar to the grain in wood although, of course, much finer and this grain runs lengthwise of the wauk. Therefore, a block constructed according to my method will present the end 25 grain to the wearing surface and in this manner act a great deal like wood, it being a well known fact that in wood the face grain wears most rapidly, the edge grain being somewhat tougher but being liable to sliver 30 off, but the end grain is extremely tough and is, therefore, used for chopping blocks and other surfaces exposed to a great amount of wear or rough usage.

In the drawings:

Fig. 1 is a perspective view of a segmental block having one roughened surface;

Fig. 2 is a view of a similar block having all of its surfaces smooth;

Fig. 3 is a perspective view of a rectangular block;

Fig. 4 is a vertical cross section of the block disclosed in Fig. 1;

Fig. 5 is a vertical cross section of the block disclosed in Fig. 2;

Fig. 6 is a vertical cross section of the block disclosed in Fig. 3;

Fig. 7 is a view showing the wauk during the process of kneading;

Fig. 8 is a view of the wauk during the

process of kneading showing the wauk folded over upon itself;

Fig. 9 is a cross section of the wauk taken on the line 9—9 of Fig. 10;

Fig. 10 is a top plan view of the finished 55 wauk;

Fig. 11 is a vertical cross section of the wauk when first inserted in a mold for making segmental blocks;

Fig. 12 is a longitudinal cross section of 60 the same;

Fig. 13 is a vertical longitudinal section of a mold with the wauk inserted for forming rectangular blocks; and

Fig. 14 is a view of the bow made use of 65 for cutting off the surplus of the wauk after the mold has been filled.

The material used is refractory material, such as fire clay and the like. This clay is first ground in a pan rather coarsely and then 70 passed through a coarse screen so as to remove extremely large lumps, after which the clay is moistened so that it assumes the approximate consistency of putty. A mass of clay is then taken and placed on a kneading 75 table 15 where the operator commences to knead it by hand so as to make the mass as homogeneous as possible. During this kneading process, what is commercially known as, a wauk 16 is formed and during the formation of this wauk a sort of grain is formed 80 therein that runs longitudinally of the wauk. After the wauk has assumed a certain length, it is folded over upon itself as disclosed in Fig. 8. This folding over, however, does not 85 materially disturb the grain except at the bent portion 17. Further kneading, however, will cause the grain to tear at this point and, again, run longitudinally of the wauk throughout its length.

It frequently happens during this folding over of the wauk that the abutting surfaces do not completely adhere. In other words they fail to unite, and I have found that where the grain runs parallel to the wearing 95 face of the block, these portions, during the removal of clinker, or ordinary wear, will chip and break out rendering the surface rough. These rough portions then wearing off cause the block to wear very readily, but 100

with my improved block such defects would run at right angles to the wearing face of the block and consequently such chipping is eliminated.

5 After the wauk has been formed, it is forcibly inserted into the mold. That is, the operator picks up the wauk and jams one end down into the mold. The mold is then bounced up and down on a table so that the 10 wauk will pack itself tightly and completely fill the mold. The bow is then brought into action and the surplus portion of the wauk is cut off therewith. This bow is of ordinary construction and consists of a curved member 18 across which is tightly stretched a wire 19 with which this cutting is done. This bow, however, is in common use and its construction is well known in the art.

20 The blocks as disclosed in Figs. 1 and 2 are for lining circular members and have arcuate faces on their wearing surface and on their surface which contacts with the wall. The block in Fig. 1 has a concave wearing surface 20 and opposite this surface a convex surface 21. These surfaces are concentric. 25 The block has parallel faces 22 and inclined faces 23. The inclined faces 23 being so inclined as to be on the radius of a circle so that by placing a predetermined number of blocks 30 together a complete circle is formed.

35 The block disclosed in Fig. 1 is for use in rotary, cement, and lime kilns, and similar structures, wherein it is desirable to build up a clinker on the interior of the lining and the block thus made merely has the surface 20 cut off by the bow thus leaving the surface 20 extremely rough so that a clinker will readily adhere thereto while the surfaces 21, 22 and 23 are troweled after the block has 40 been removed from the mold to make them perfectly smooth.

45 In the construction of the block, in Fig. 2 the surfaces 24, 25, 26 and 27 are made in the same manner as the surfaces disclosed in Fig. 1, with this exception, that the surface 24 is also troweled so as to render it smooth. This block is to be used in circular construction where the adherence of clinker is not wanted.

50 The block disclosed in Fig. 3 is rectangular and is designed to have the surfaces either 28 or 29 be the wearing surface.

55 In all of these constructions, as described, the grain of the various blocks will run at right angles to the wearing surface, that is, in Fig. 1 the grain will run at right angles to the faces 20 and 21; in Fig. 2 at right angles to the faces 24 and 25; and in Fig. 3 to the faces 28 and 29 so that when the blocks are 60 used, the end grain will be exposed.

65 In Figs. 11 and 12 I have shown molds for making segmental blocks for circular casings. These molds preferably consist of a body portion 30 and a bottom 31, the bottom 31 forming the convex surface of the block.

The body portion 30 is preferably provided with ears 32 and the bottom with ears 33 so that the mold can be assembled by means of screw or C clamps 34. These clamps not only secure the bottom in position but also act as handles when the mold is bounced on the table for packing the wauk in the mold. Of course, it is to be understood that the mold, either as disclosed in Figs. 11 and 12 or in Fig. 13, is so constructed that a certain amount of air leakage can occur. This is to permit the wauk to fully fill the mold and without the formation of air pockets in the corners.

70 When a rectangular block, as disclosed in Fig. 3, is made, a mold 35 is employed. This may be either a two-piece mold so that the bottom 36 can be removed, or it may be a one-piece mold. The bouncing of the molds, as previously described, not only fills out the corners of the mold completely but also has a tendency to pack material and render it still more dense within the mold but it does not in any way change the trend of the grain, which has been worked up in the wauk.

75 My blocks, and method of making the same, are directed to hand made blocks only, that is a block made of clay which has been kneaded by hand because I have found that hand made blocks and, especially when made by my improved method, are tougher and last much longer than where the wauk is squeezed out from an auger machine because the auger, in squeezing out the clay, cuts through the grain so that the resulting block has the grain running in various directions and there is no possible way in which end grain can be positively obtained at the wearing face of blocks made in an auger machine.

80 Furthermore I have found that the trade 105 is willing to pay more for a hand-made block than for machine-made blocks on account of their longer life and especially in view of the fact that there is less possibility of air pockets being formed in the block when hand made than in machine-made blocks. In other words, the hand-made block is more homogeneous and really denser in a way than a machine-made block even though the block 110 has been made on a press because the kneading of the wauk under the hands of a skilled workman will obviate air pockets and make the mass of a more uniform density throughout.

85 While I have previously disclosed grinding the clay while dry and then screening it before moistening the same, I may, in order to save time, grind the same in what is called a wet pan. In this pan the mulls are set at a predetermined distance above the bottom 120 of the pan, this regulating the fineness of the grinding. The clay is put into the pan and ground for a predetermined length of time so as to reduce the large lumps. The grinding is then continued and water added 125

5 during the grinding so as to reduce the mass to the proper consistency. After this the grinding is continued without the addition of any further water until all particles are thoroughly mixed. It is then removed from the pan and kneaded in the usual manner. By thus preparing the clay, considerable time is saved and the results obtained are equal in every respect to where the clay is ground 10 dry and screened.

10 The clay used in the manufacture of my blocks has preferably an alumina content of at least fifty (50%) per cent.

15 While I have described the block as being made of rough material and having its wearing face finished by means of a bowd, I do not desire to limit myself thereto as I can make a perfectly smooth block and after removing it from the mold scarify or roughen 20 the wearing face in any well known manner.

25 Another point I desire to stress is that the content of my block contains silica and alumina which, when subjected to a high temperature, will combine and form silicate of alumina, commonly known as mullite.

30 Therefore, blocks made by my method will contain mullite when subjected to a sufficiently high temperature, which will aid in lengthening the life of the block because it 35 resists expansion and contraction. While I have stated that the grain formed in the blocks preferably runs at right angles to the wearing face, this is not essential as any angle less than a right angle and greater than parallel will be suitable and will toughen the wearing face of the block.

Having fully described my invention, what I claim is:

1. The method of making refractory blocks 40 which consists in hand kneading a wauk of refractory clay, separating a portion of said wauk from the remainder thereof and then giving to said separated portion the desired shape in such a manner that the grain formed 45 therein during the kneading will extend at right angles to the wearing face of the block.

2. The method of making refractory blocks 50 which consists in kneading a wauk of plastic fire clay so as to establish therein a grain extending longitudinally of the wauk and then forming the wauk into blocks having the grain extending at right angles to the wearing face of said blocks.

3. The method of making refractory blocks 55 which consists in kneading a wauk of moistened fire clay so as to establish a longitudinally extending grain therein, placing said wauk in a mold with the grain of the wauk at right angles to the bottom of the 60 mold, removing the surplus clay from the top of the mold thereby forming a wearing face with the grain running at right angles thereto, and then removing said block from said mold.

4. The method of making refractory blocks

which consists in kneading a wauk of moistened fire clay so as to establish a longitudinally extending grain therein, placing said wauk in a mold with the grain of the wauk at right angles to the bottom of the 70 mold, removing the surplus clay from the top of the mold thereby forming a wearing face with the grain running at right angles thereto, then removing said block from said mold, and lastly, smoothing the faces of said block.

5. The method of making refractory blocks 75 which consists in kneading a wauk of moistened fire clay so as to establish a longitudinally extending grain therein, placing said wauk in a mold with the grain of the wauk at right angles to the bottom of the mold, removing the surplus clay from the top of the mold thereby forming a wearing face with the grain running at right angles thereto, then removing said block from said mold, and lastly, smoothing all the faces of said block except the wearing face.

6. The method of making refractory blocks 80 which consists in crushing dry fire clay, passing said crushed clay through a screen so as to remove the larger lumps therefrom forming said clay into a plastic mass by the addition of water, kneading said plastic mass of clay into a wauk so as to establish a grain 85 therein running longitudinally of the wauk, placing said wauk in a mold with the grain thereof running at right angles to the bottom thereof, packing said clay into said mold so as to render the same more dense and without disturbing the trend of the grain, removing the surplus clay from the top of the mold thereby forming a wearing face with the grain running at right angles thereto, and, 90 lastly, removing said block from said mold.

7. The method of making refractory blocks 95 which consists in crushing a quantity of fire clay, passing said ground clay through a screen so as to remove the larger lumps thereof, adding water to said clay so as to form a plastic mass, kneading said clay into a wauk 100 so as to establish a grain therein running longitudinally of the wauk, placing said wauk in a mold with the grain running at right angles to the bottom thereof, packing said clay into said mold so as to render the same more dense and without disturbing the trend of the grain, removing the surplus clay from the top of the mold thereby forming 105 a wearing face on the block with the grain running at right angles thereto, removing said block from said mold, and lastly, smoothing the remaining faces of said block.

8. The method of making refractory blocks 110 which consists in crushing a body of fire clay, removing the larger lumps therefrom adding water to said clay so as to form a plastic mass, kneading said clay into a wauk in such a manner as to establish a grain therein running 115 longitudinally of the wauk, placing said wauk 120

in a mold with the grain running at right angles to the bottom thereof, packing said clay into said mold so as to render the same more dense and without disturbing the trend of the grain, removing the surplus clay from the top of the mold thereby forming a wearing face with the grain running at right angles thereto, removing said block from said mold, and lastly, smoothing all of the faces of said block except the wearing face.

10 9. The method of making refractory blocks which consists in kneading a wauk of plastic fire clay containing silica and alumina so as to establish a grain therein and extending longitudinally of said wauk, forming the wauk into blocks having the grain of the wauk at right angles to the wearing face of said blocks, and then exposing said blocks to a high temperature thereby causing said 15 silica and alumina content to combine to form mullite therein.

20 In testimony whereof I have affixed my signature.

GEORGE W. PARKER.

25

30

35

40

45

50

55

60

65